



US006695934B1

(12) **United States Patent**  
**Bhargava**

(10) **Patent No.:** **US 6,695,934 B1**  
(45) **Date of Patent:** **\*Feb. 24, 2004**

(54) **COPPER ALLOY AND PROCESS FOR OBTAINING SAME**

(75) Inventor: **Ashok K. Bhargava**, Cheshire, CT (US)

(73) Assignee: **Waterbury Rolling Mills, Inc.**, Waterbury, CT (US)

(\*) Notice: Subject to any disclaimer, the term of this patent is extended or adjusted under 35 U.S.C. 154(b) by 0 days.

This patent is subject to a terminal disclaimer.

(21) Appl. No.: **09/527,144**

(22) Filed: **Mar. 16, 2000**

**Related U.S. Application Data**

(60) Continuation of application No. 09/103,866, filed on Jun. 24, 1998, now Pat. No. 6,099,663, which is a division of application No. 08/931,696, filed on Sep. 16, 1997, now Pat. No. 5,893,953.

(51) **Int. Cl.<sup>7</sup>** ..... **C22C 9/04**

(52) **U.S. Cl.** ..... **148/434; 148/433; 420/472; 420/473; 420/476**

(58) **Field of Search** ..... **148/433, 434; 420/476, 472, 499, 473, 496**

(56) **References Cited**

**U.S. PATENT DOCUMENTS**

4,822,562 A \* 4/1989 Miyafuji et al. ..... 420/472

4,971,758 A \* 11/1990 Suzuki et al. ..... 420/472  
5,024,814 A 6/1991 Futatasuka et al. ..... 420/473  
5,508,001 A \* 4/1996 Suzuki et al. ..... 420/472  
5,624,506 A 4/1997 Tsuzaki et al. ..... 148/433  
6,099,663 A \* 8/2000 Bhargava ..... 148/434

**FOREIGN PATENT DOCUMENTS**

|    |           |          |
|----|-----------|----------|
| JP | 62-116745 | * 5/1987 |
| JP | 03-294461 | 4/1990   |
| JP | 06-073474 | 8/1992   |
| JP | 06-220594 | 1/1993   |
| JP | 10-130755 | 11/1996  |

\* cited by examiner

*Primary Examiner*—John Sheehan

(74) *Attorney, Agent, or Firm*—Wiggin & Dana LLP; William A. Simons; Michael K. Kinney

(57) **ABSTRACT**

A copper base alloy consisting essentially of tin in an amount from about 0.1 to about 1.5% by weight, phosphorous in an amount from about 0.01 to about 0.35% by weight, iron in an amount from about 0.01 to about 0.8% by weight, zinc in an amount from about 1.0 to about 15% by weight, and the balance essentially copper, including phosphide particles uniformly distributed throughout the matrix, is described. The alloy is characterized by an excellent combination of physical properties. The process of forming the copper base alloy described herein includes casting, homogenizing, rolling, process annealing and stress relief annealing.

**20 Claims, No Drawings**

## COPPER ALLOY AND PROCESS FOR OBTAINING SAME

This is a Continuation of application Ser. No. 09/103, 866, filed Jun. 24, 1998, now U.S. Pat. No. 6,099,663 which is a divisional application of application Ser. No. 08/931,696 filed Jan. 16, 1997, now U.S. Pat. No. 5,893,953.

### CROSS-REFERENCE TO RELATED APPLICATION(S)

The present application is related to U.S. patent application Ser. No. 08/747,014, filed Nov. 7, 1996, entitled COPPER ALLOY AND PROCESS FOR OBTAINING SAME and to U.S. patent application Ser. No. 08/780,116, filed Dec. 26, 1996, entitled COPPER ALLOY AND PROCESS FOR OBTAINING SAME.

### BACKGROUND OF THE INVENTION

The present invention relates to copper base alloys having utility in electrical applications and to a process for producing said copper base alloys.

There are a number of copper base alloys that are used in connector, lead frame and other electrical applications because their special properties are well suited for these applications. Despite the existence of these alloys, there remains a need for copper base alloys that can be used in applications that require high yield strength greater than 80 KSI, together with good forming properties that allow one to make 180° badway bends with a R/T ratio of 1 or less plus low relaxation of stress at elevated temperatures and freedom of stress corrosion cracking. Alloys presently available do not meet all of these requirements or have high costs that make them less economical in the marketplace or have other significant drawbacks. It remains highly desirable to develop a copper base alloy satisfying the foregoing goals.

Beryllium copper generally has very high strength and conductivity along with good stress relaxation characteristics; however, these materials are limited in their forming ability. One such limitation is the difficulty with 180° badway bends. In addition, they are very expensive and often require extra heat treatment after preparation of a desired part. Naturally, this adds even further to the cost.

Phosphor bronze materials are inexpensive alloys with good strength and excellent forming properties. They are widely used in the electronic and telecommunications industries. However, they tend to be undesirable where they are required to conduct very high current under very high temperature conditions, for example under conditions found in automotive applications for use under the hood. This combined with their high thermal stress relaxation rate makes these materials less suitable for many applications.

High copper, high conductivity alloys also have many desirable properties, but generally do not have mechanical strength desired for numerous applications. Typical ones of these alloys include, but are not limited to, copper alloys 110, 122, 192 and 194.

Representative prior art patents include U.S. Pat. Nos. 4,666,667, 4,627,960, 2,062,427, 4,605,532, 4,586,967, 4,822,562, and 4,935,076.

Accordingly, it is highly desirable to develop copper base alloys having a combination of desirable properties making them eminently suitable for many applications.

### SUMMARY OF THE INVENTION

In accordance with the present invention, it has been found that the foregoing objective is readily obtained.

Copper base alloys in accordance with the present invention consist essentially of tin in an amount from about 0.1 to about 1.5%, preferably from about 0.4 to 0.9%, phosphorous in an amount from about 0.01 to about 0.35%, preferably from about 0.01% to about 0.1%, iron in an amount from about 0.01% to about 0.8%, preferably from about 0.05% to about 0.25%, zinc in an amount from about 1.0 to about 15%, preferably from about 6.0 to about 12.0%, and the balance essentially copper. It is particularly advantageous to include nickel and/or cobalt in an amount up to about 0.5% each, preferably in an amount from about 0.001% to about 0.5% each. Alloys in accordance with the present invention may also include up to 0.1% each of aluminum, silver, boron, beryllium, calcium, chromium, indium, lithium, magnesium, manganese, lead, silicon, antimony, titanium, and zirconium. As used herein, the percentages are weight percentages.

It is desirable and advantageous in the alloys of the present invention to provide phosphide particles of iron and/or nickel and/or magnesium or a combination thereof, uniformly distributed throughout the matrix since these particles serve to increase strength, conductivity, and stress relaxation characteristics of the alloys. The phosphide particles may have a particle size of 50 Angstroms to about 0.5 microns and may include a finer component and a coarser component. The finer component may have a particle size ranging from about 50 to 250 Angstroms, preferably from about 50 to 200 Angstroms. The coarser component may have a particle size generally from 0.075 to 0.5 microns, preferably from 0.075 to 0.125 microns.

The alloys of the present invention enjoy a variety of excellent properties making them eminently suitable for use as connectors, lead frames, springs and other electrical applications. The alloys should have an excellent and unusual combination of mechanical strength, formability, thermal and electrical conductivities, and stress relaxation properties.

The process of the present invention comprises: casting a copper base alloy having a composition as aforesaid; 40 homogenizing at least once for at least one hour at temperatures from about 1000 to 1450° F.; rolling to finish gauge including at least one process anneal for at least one hour at 650 to 1200° F.; and stress relief annealing for at least one hour at a temperature in the range of 300 to 600° F., thereby obtaining a copper alloy including phosphide particles uniformly distributed throughout the matrix. Nickel and/or cobalt may be included in the alloy as above.

### DETAILED DESCRIPTION OF THE PREFERRED EMBODIMENT(S)

The alloys of the present invention are modified copper-tin-zinc alloys. They are characterized by higher strengths, better forming properties, higher conductivity, and stress relaxation properties that represent a significant improvement over the same properties of the unmodified alloys.

The alloys in accordance with the present invention include those copper base alloys consisting essentially of tin in an amount from about 0.1 to 1.5%, preferably from about 0.4 to about 0.9%, phosphorous in an amount from about 0.01 to about 0.35%, preferably from about 0.01 to about 0.1%, iron in an amount from about 0.01 to about 0.8%, preferably from about 0.05 to about 0.25%, zinc in an amount from about 1.0 to about 15%, preferably from about 6.0 to about 12.0%, and the balance essentially copper. These alloys typically will have phosphide particles uniformly distributed throughout the matrix.

These alloys may also include nickel and/or cobalt in an amount up to about 0.5% each, preferably from about 0.001 to about 0.5% of one or combinations of both.

One may include one or more of the following elements in the alloy combination: aluminum, silver, boron, beryllium, calcium, chromium, indium, lithium, magnesium, manganese, lead, silicon, antimony, titanium, and zirconium. These materials may be included in amounts less than 0.1%, each generally in excess of 0.001 each. The use of one or more of these materials improves the mechanical properties such as stress relaxation properties; however, larger amounts may affect conductivity and forming properties.

The aforesaid phosphorous addition allows the metal to stay deoxidized making it possible to cast sound metal within the limits set for phosphorous, and with thermal treatment of the alloys, phosphorous forms a phosphide with iron and/or iron and nickel and/or iron and magnesium and/or a combination of these elements, if present, which significantly reduces the loss in conductivity that would result if these materials were entirely in solid solution in the matrix. It is particularly desirable to provide iron phosphide particles uniformly distributed throughout the matrix as these help improve the stress relaxation properties by blocking dislocation movement.

Iron in the range of about 0.01 to about 0.8% and particularly about 0.05 to about 0.25% increases the strength of the alloys, promotes a fine grain structure by acting as a grain growth inhibitor and in combination with phosphorous in this range helps improve the stress relaxation properties without negative effect on electrical and thermal conductivities.

Nickel and/or cobalt in an amount from about 0.001 to 0.5% each are desirable additives since they improve stress relaxation properties and strength by refining the grain and through distribution throughout the matrix, with a positive effect on the conductivity.

The process of the present invention includes casting an alloy having a composition as aforesaid. Any suitable casting technique known in the art such as horizontal continuous casting may be used to form a strip having a thickness in the range of from about 0.500 to 0.750 inches. The processing includes at least one homogenization for at least one hour, and preferably for a time period in the range of from about 1 to about 24 hours, at temperatures in the range of from about 1000 to 1450° F. At least one homogenization step may be conducted after a rolling step. After homogenization, the strip may be milled once or twice to remove from about 0.020 to 0.100 inches of material from each face.

The material is then rolled to final gauge, including at least one process anneal at 650 to 1200° F. for at least one hour and preferably for about 1 to 24 hours, followed by slow cooling to ambient at 20 to 200° F. per hour.

The material is then stress relief annealed at final gauge at a temperature in the range of 300 to 600° F. for at least one hour and preferably for a time period in the range of about 1 to 20 hours. This advantageously improves formability and stress relaxation properties.

The thermal treatments advantageously and most desirably provide the alloys of the present invention with phosphide particles of iron and/or nickel and/or magnesium or a combination thereof uniformly distributed throughout the matrix. The phosphide particles increase the strength, conductivity, and stress relaxation characteristics of the alloys. The phosphide particles may have a particle size of about 50 Angstroms to about 0.5 microns and may include a finer component and a coarser component. The finer

component may have a particle size of about 50 to 250 Angstroms, preferably from about 50 to 200 Angstroms. The coarser component may have a particle size generally from 0.075 to 0.5 microns, preferably from 0.075 to 0.125 microns.

Alloys formed in accordance with the process of the present invention and having the aforesaid compositions are capable of achieving a yield strength in the 80-100 ksi range with bending ability at a radius equal to its thickness, 10 badway, on a width up to 10 times the thickness. Additionally, they are capable of achieving an electrical conductivity of the order of 35% IACS, or better. The foregoing coupled with the desired metallurgical structure should give the alloys a high stress retention ability, for 15 example over 60% at 150° C., after 1000 hours with a stress equal to 75% of its yield strength on samples cut parallel to the direction of rolling, and makes these alloys very suitable for a wide variety of applications requiring high stress retention capabilities. Moreover, the present alloys do not 20 require further treatment by stampers.

This invention may be embodied in other forms or carried out in other ways without departing from the spirit or essential characteristics thereof. The present embodiments are therefore to be considered as in all respects illustrative 25 and not restrictive, the scope of the invention being indicated by the appended claims, and all changes which come within the meaning and range of equivalency are intended to be embraced therein.

What is claimed is:

30 1. A copper base alloy having a matrix, said alloy consisting of tin in an amount from about 0.1 to about 1.5% by weight, phosphorous in an amount from about 0.01 to about 0.35% by weight, iron in an amount from about 0.01 to about 0.8% by weight, zinc in an amount from about 1.0 to about 15% by weight, and the balance essentially copper, said alloy including phosphide particles uniformly distributed throughout the matrix, said phosphide particles including a finer component made up of phosphide particles having a size in the range of from about 50 to about 250 Angstroms and a coarser component made up of phosphide particles having a size in the range of from about 0.075 to about 0.5 microns.

35 2. A copper base alloy according to claim 1, wherein said tin content is from about 0.4 to about 0.9% by weight.

40 3. A copper base alloy having a matrix, said alloy consisting of tin in an amount from about 0.1 to 1.5% by weight, phosphorous in an amount from about 0.01 to about 0.35% by weight, iron in an amount from about 0.01 to 0.8% by weight, zinc in an amount from about 1.0 to about 15% by weight, a material selected from the group consisting of nickel, cobalt and mixtures thereof in an amount from about 0.001 to 0.5% by weight each, and the balance essentially copper, said alloy including phosphide particles uniformly distributed throughout the matrix, and said phosphide particles including a finer component made up of phosphide particles having a size in the range of from about 50 to about 250 Angstroms and a coarser component made up of phosphide particles having a size in the range of from about 0.075 to about 0.5 microns.

45 4. A copper base alloy having a matrix, said alloy consisting of tin in an amount from about 0.1 to 1.5% by weight, phosphorous in an amount from about 0.01 to about 0.35% by weight, iron in an amount from about 0.01 to 0.8% by weight, zinc in an amount from about 1.0 to about 15% by weight, at least one addition selected from the group consisting of aluminum, silver, boron, beryllium, calcium, chromium, indium, lithium, magnesium, manganese, lead, 50

silicon, antimony, titanium and zirconium, said at least one addition being present in an amount up to 0.1% each, and the balance essentially copper, said alloy including phosphide particles uniformly distributed throughout the matrix, and said phosphide particles including a finer component made up of phosphide particles having a size in the range of from about 50 to about 250 Angstroms and a coarser component made up of phosphide particles having a size in the range of from about 0.075 to about 0.5 microns.

5. A copper base alloy according to claim 1, wherein said phosphorous content is from about 0.01 to about 0.10% by weight.

6. A copper base alloy according to claim 1, wherein said iron content is from about 0.05 to about 0.25% by weight.

7. A copper base alloy according to claim 1, wherein said finer component is made up of phosphide particles having a size in the range of 50 to 200 Angstroms and said coarser component is made up of phosphide particles having a size in the range of 0.075 to 0.125 microns.

8. A copper base alloy having a matrix and consisting of tin in an amount from about 0.1 to about 1.5% by weight, phosphorous in an amount from about 0.01 to about 0.35% by weight, iron in an amount from about 0.01 to about 0.8% by weight, zinc in an amount from about 1.0 to about 15% by weight, a material selected from the group consisting of nickel, cobalt and mixtures thereof in an amount from 0.001 to 0.5% by weight each, magnesium in an amount up to 0.1% by weight, at least one addition selected from the group consisting of aluminum, silver, boron, beryllium, calcium, chromium, indium, lithium, manganese, lead, silicon, antimony, titanium, and zirconium, said at least one addition being present in an amount up to 0.1% each, and the balance copper, said alloy including phosphide particles uniformly distributed throughout the matrix, said phosphide particles including a finer component made up of phosphide particles having a size in the range of from about 50 to about 250 Angstroms and a coarser component made up of phosphide particles having a size in the range of from about 0.075 to about 0.5 microns.

9. A copper base alloy according to claim 8, wherein said phosphide particles are selected from the group consisting of iron nickel phosphide particles, iron magnesium phosphide particles, iron phosphide particles, magnesium nickel phosphide particles, magnesium phosphide particles and mixtures thereof.

10. A copper base alloy according to claim 8, wherein said zinc is present in an amount from about 6.0 to 12.0% by weight.

11. A copper base alloy according to claim 8, wherein said phosphorous content is from 0.01 to about 0.10 by weight.

12. A copper base alloy according to claim 8, wherein said iron content is from about 0.05% to about 0.25% by weight.

13. A copper base alloy according to claim 8, wherein said tin content is from about 0.4% to about 0.9% by weight.

14. A copper base alloy according to claim 8, wherein said zinc content is greater than 6% by weight.

15. A copper base alloy having a matrix which comprises phosphide particles uniformly distributed throughout said matrix, said phosphide particles including a finer component made up of phosphide particles having a size in a range of from about 50 to about 250 Angstroms and a coarser component made up of phosphide particles having a size in a range of from about 0.075 to about 0.5 microns, said phosphide particles formed within said matrix by casting said alloy consisting of tin in an amount from about 0.1 to about 1.5% by weight, phosphorous in an amount from about 0.01 to about 0.35% by weight, iron in an amount from about 0.01 to about 0.8% by weight, zinc in an amount from about 1.0 to about 15% by weight, and the balance essentially copper, wherein said alloy is prepared by a process comprising, homogenizing said alloy for at least one hour at a temperature in a range of about 1000 to 1450° F.; rolling to final gauge, said rolling to final gauge step including at least one process annealing step for at least one hour at a temperature of range of about 650 to 1200° F., followed by slow cooling to ambient at 20 to 200° F. per hour, and then stress relief annealing for at least one hour at a temperature in a range of about 300 to 600° F.

16. The copper base alloy of claim 15 wherein said finer component of said phosphide particles having a size in a range of from about 50 to about 200 Angstroms.

17. The copper base alloy of claim 15 wherein said coarser component of said phosphide particles having a size in a range of from about 0.075 to about 0.125 microns.

18. The copper base alloy of claim 15 wherein the homogenizing step is performed for a time period in a range of from about 1 to 24 hours.

19. The copper base alloy of claim 15 wherein the process annealing step in the rolling to final gauge step is performed for a time period in a range of from about 1 to 24 hours.

20. The copper base alloy of claim 15 wherein the stress relief annealing step is performed for a time period in a range of from about 1 to 20 hours.

\* \* \* \* \*